

Oct. 6, 1925.

1,555,915

R. ELLIS

## SEPARATING PROCESS

Filed March 9, 1925



*Witness.*

John G. Andrew

Inventor  
Ridsdale Ellis  
By Leonard Murray  
his attorney.

## UNITED STATES PATENT OFFICE.

RIDSDALE ELLIS, OF OAK PARK, ILLINOIS.

## SEPARATING PROCESS.

Application filed March 9, 1925. Serial No. 14,209.

*To all whom it may concern:*

Be it known that I, RIDSDALE ELLIS, a citizen of the United States, and a resident of Oak Park, in the county of Cook and State of Illinois, have invented certain new and useful Improvements in Separating Processes, of which the following is a specification.

My invention relates to processes for concentrating ores and other materials by means of froth flotation and the like.

This application is a continuation in part of my co-pending application Serial Number 345,137, filed December 15, 1919, which application was a renewal of application Serial Number 271,349, filed January 16, 1919.

The principal objects of my invention are in general to enhance the efficiency of such separating processes as hitherto carried out, more particularly by means of certain gases, and generally to improve the separation of comminuted materials by flotation.

I have found that whereas in froth flotation emulsification and flotation are normally carried out in an atmosphere of ordinary air superior results are obtainable by the use of other gases more particularly oxygen.

I have further found that while an atmosphere of oxygen is useful in both emulsification and flotation the advantageous results obtained are nearly as great when oxygen is used in the emulsification treatment only.

While the mixing of the ore with the modifying agent is the primary purpose of the emulsification treatment such treatment also involves aeration of the ore pulp, aeration also takes place to a more limited extent in the tube mill or other grinding apparatus which may be employed.

The precise cause of the beneficial effects produced by the use of oxygen in place of air and of air in place of nitrogen are uncertain. It is believed, however, that one of the factors involved is the contact and other electrical effects occurring at the gas-water, gas-particle and other interfaces.

Suitable electrical conditions favor the adhesion and it has been found that chemical action either complete or incipient greatly increases the electrification of gases. Thus a gas bubble generated chemically in water is much more highly charged than one intro-

duced bodily from the surrounding atmosphere.

Now of the constituents of air only one is chemically active, viz oxygen, and I have found that this constituent is the active one in flotation, the extraction of a zinc ore, for example, being much higher in an atmosphere of oxygen than in one of air.

Further I have found that in certain cases of ozonizing the air in which the ore pulp is agitated aids the extraction, especially when the quantity of frothing agent is small.

Substantially pure oxygen is, however, ordinarily superior to ozonized air which necessarily contains all of the nitrogen contained in the original air.

I have also found that the advantageous results obtainable by the use of oxygen in place of air are much more marked in the case of a relatively difficultly floatable material, like zinc sulphide, than in the case of relatively easily floatable material, like copper sulphide.

In practice carried out by me on a zinc-lead ore assaying about 18% of zinc I have found that by mechanically agitating the ore pulp in an atmosphere of oxygen instead of air the percentage of zinc remaining in the tails was reduced about 50% when both emulsification and aeration take place in oxygen and about 35% when only emulsification is carried out in an atmosphere of oxygen.

It will be understood that in addition to oxygen any suitable reagents may be employed, such as copper sulphate and sulphuric acid in the case of zinc ores.

Further, a soluble frothing agent may be employed in place of the oil either wholly or in part. Similarly a frothing agent in vapor form may be used in place of or in addition to the liquid oil as soluble frothing agent.

The various forms of apparatus commonly employed for carrying out the separation of metalliferous matter by flotation are so well known to those skilled in the art that the diagrammatical sectional illustration in the drawings of a flotation machine of the mechanical agitation type will suffice.

The apparatus comprises an emulsifier cell 1, a frothing cell 2 and a separating chamber or spitzkasten 3. In the emulsifier cell 1, an agitator 4 is provided, mounted at the

end of a shaft 5, rotated by means of a shaft 6, connected thereto by means of bevel gears 7 and 8. The ore pulp is fed into the emulsifier through the pipe 9. Oil is fed into the 5 emulsifier through the pipe 10. As a result of the agitation in the emulsifier the metalliferous particles in the ore pulp become coated with the oil and then the ore pulp passes through the passage 11 into the frothing cell 10. 2. In the latter is arranged an agitator 12 mounted on a shaft 13 driven from the shaft 6 by means of bevel gears 14 and 15.

The lower part of the cell 2 is connected with the spitzkasten by an aperture 16 15 through which passes the ore pulp after being aerated in the cell 2. In the spitzkasten the gangue sinks to the bottom while the metalliferous matter adhering to bubbles of gas are rafted to the surface of the pulp to 20 form a layer of froth 17 on the surface of the water. The froth flows over a lip 18 into the launder 19 from which the concentrates including any froth which has not been broken down in the launder may be 25 withdrawn through pipe 20.

The tails, consisting of silica, silicates, etc., sink to the bottom of the spitzkasten 3 and collect in the hopper-shaped part 21 from which they may be sent by pipe 22 either to 30 the tailing pond or else to a second chamber for further treatment.

In order that the ore may be mixed with the modifying or frothing agent in an atmosphere of oxygen or a gaseous mixture containing a higher percentage of oxygen than air the upper part of the emulsifier 1, is enclosed by a cover 23. A gas inlet pipe 24 and outlet pipe 25 are provided so that oxygen may be admitted and exhausted 40 after it has become diluted with nitrogen or other gases released from solution in the water of the ore pulp.

Preferably the upper part of the frothing cell 2, is similarly enclosed at 26 and oxygen 45 supplied thereto by means of a pipe 27. The oxygen from the frothing cell may conveniently be discharged into the inlet pipe 24 of the emulsifier. This counter current arrangement is preferred as the greatest contamination of oxygen by nitrogen from the water in the ore pulp will be in the emulsifier.

While I have illustrated and described my invention in connection with the mechanical 55 agitation froth process it may also be used in connection with the pneumatic agitation process, as well as processes of other types, more particularly those in which the gas bubbles are generated in the ore pulp instead 60 of being introduced into the latter from a previously formed body of gas.

Oxygen may be generated in the ore pulp by dissolving it in the water and then liberating it by the action of heat or pressure reduction, by chemical reaction, by the decom-

position of such substances as hydrogen peroxide or by electrolysis or similar means.

Further, while ordinarily oxygen used in connection with a mechanical agitation froth apparatus is generated outside of the pulp 70 it is not essential to do so and the necessary supply of oxygen may be formed in the pulp by electrolysis or other means.

I am aware that numerous details of the process may be varied through a wide range 75 without departing from the spirit of this invention, and I do not desire limiting the patent granted otherwise than as necessitated by the prior art.

I claim:

1. The process of concentrating ores by flotation which includes mixing the ore pulp with a modifying agent, aerating the pulp to form a froth and separating the froth from the remainder by flotation, and which further includes the use of an externally prepared gas containing more than 25% free oxygen by volume for aiding in the formation of the froth.

2. The process of concentrating ores by flotation which includes mixing the ore pulp with a modifying agent, aerating the pulp at substantially atmospheric pressure to form a froth and separating the froth from the remainder by flotation, and which further includes subjecting the ore pulp to a gas containing more than 25% free oxygen by volume during said mixing step.

3. The process of concentrating ores by flotation which includes mixing the pulp with a modifying agent to coat the mineral particles, aerating the pulp at substantially atmospheric pressure to form a froth and separating the froth from the remainder by flotation, and which further includes the use of a gas containing more than 25% free oxygen by volume for aiding in the coating of the particles.

4. The process of concentrating ores which includes aerating the pulp with an externally prepared gas containing more than 25% free oxygen by volume to form a froth, and separating the mineral carried by the froth from the remainder of the ore.

5. The process of concentrating ores which includes producing bubbles of gas in the ore pulp to form a froth, substantially all of which bubbles contain over 40% free oxygen by volume, and separating the mineral carried by the froth from the remainder of the ore.

6. The process of concentrating ores by flotation which includes mixing the ore pulp with a modifying agent, aerating the pulp to form a froth and separating the froth from the remainder by flotation, and which further includes the use of a gas containing more than 40% free oxygen by volume for aiding in the formation of the froth.

7. The process of concentrating ores by

flotation which includes mixing the ore pulp with a modifying agent to coat the mineral particles, aerating the pulp to form a froth, and separating the froth from the remainder by flotation, and which further includes the use of a gas containing more than 5 40% free oxygen by volume for aiding in the coating of the particles.

8. The process of concentrating ores which 10 includes mixing the ore pulp with a modifying agent, aerating the pulp with an externally prepared gas having a substantially greater direct oxidizing power than atmospheric air to form a froth, and separating the mineral carried by the froth 15 from the remainder of the ore,

9. The process of concentrating ores which includes mixing the ore pulp with a modi-

fying agent to coat the metalliferous particles, aerating the ore pulp at substantially 20 atmospheric pressure to form a froth and separating the froth from the remainder by flotation and which further includes the use of a gas having a substantially greater oxidizing power than atmospheric air to aid in 25 the coating of the particles.

10. The process of concentrating ores by flotation which includes mixing the ore pulp with a modifying agent, aerating the pulp to form a froth and separating the froth 30 from the remainder by flotation, and which further includes the use of substantially pure oxygen for aiding in the formation of a froth.

RIDSDALE ELLIS.